

1

2,899,392

## PROCESS OF REDUCING THE CONSISTENCY OF SOLID-AND-LIQUID MIXTURES

Hubert Schranz, Clausthal-Zellerfeld, Germany, assignor to Metallgesellschaft A.G., Frankfurt am Main, Germany

No Drawing. Application September 12, 1955  
Serial No. 533,905

Claims priority, application Germany September 17, 1954

4 Claims. (Cl. 252—60)

This invention relates to a process for reducing the consistency of solid-and-liquid mixtures, which is applicable to various industrial purposes in which it is desired either to reduce the consistency of such mixture for a given solids content or to increase the solids content of a solid-and-liquid mixture with the same or even reduced final consistency.

The possibility of increasing the fluidity of a thick or pasty suspension or of increasing its solids content and specific gravity without obtaining an inadmissibly thick suspension is of special importance in the heavy-media separation of minerals, such as ore and coal.

Aqueous suspensions of finely ground heavy solids, as a rule of ferrosilicon, magnetite, galena, pyrite, quartz, barium sulphate, or the like, are used for preparing the heavy medium in which the separation is effected in said classifying processes.

Heavy media made with these substances have the disadvantage, however, that their consistency (apparent viscosity) increases progressively with an increase in their content of heavy solids, i.e. with an increase in specific gravity, so that the specific gravity of heavy media having a consistency which is compatible with a perfect float and sink process cannot be increased in practice beyond approximately half the specific gravity of the heavy solid used because otherwise the lighter particles of the material to be classified will no longer float since in most mineral mixtures to be subjected to heavy-media separation the difference between the specific gravities of the components to be separated is not too great. For this reason it has previously been necessary to use heavy solids of very high specific gravity.

The resulting difficulties and disadvantages are removed according to the invention thereby that small quantities of certain interface-active substances are added to the media, whereby the consistency of the suspensions is reduced in such a degree that a considerable increase in the volume share of the heavy solid is possible, e.g., in making a heavy medium for classification purposes. In many cases this enables also the preparation of suspensions having the specific gravity required for the separation while using comparatively light-weight heavy solids. For instance, it is now possible to use as heavy media suspensions whose heavy solids consist of one or several heavy components of the mineral mixture to be classified. A suspension of barium sulphate can be used, e.g., for separating a mixture of barium sulphate and quartz. According to the new process the consistency of said mixture is in spite of its high content of solids reduced far enough to ensure a perfect separation with reference to the specific gravity.

Another advantage of the invention resides in the fact that in most cases the addition of the surface-active agents will considerably increase the stability of the suspension compared to one that has not been treated according to the invention. This is due to the fact that

2

the equipolar electric charging of the solid particles suspended in the liquid is increased by the interface-active substances added.

This effect of the new process may be decisive for its application even where the reduction of the consistency is not critical.

Interface-active substances suitable for the purpose of the invention include cationic compounds of the series consisting of the fatty amines and their salts, preferably fatty amines  $C_nH_{2n+1}NH_2$  and their salts  $C_nH_{2n+1}NH_3Cl$  (chloride) and  $C_nH_{2n+1}NH_3OOC—CH_3$  (acetate), such as stearylamine  $C_{18}H_{37}NH_2$ , stearylamine acetate  $C_{18}H_{37}NH_3OOC—CH_3$  and stearylamine hydrochloride  $C_{18}H_{37}NH_3Cl$  or coconut amine, tallow amine and their salts. In the formulae given the index  $n$  states the number of carbon atoms in the molecule; the compounds concerned have between about 6 and 18 carbon atoms in the molecule, i.e.  $n$ =between 6 and 18.

The proportions in which said substances are added are only small in all cases. The optimum quantities can be easily determined. Generally they are between 1–20 kg./m.<sup>3</sup>, depending on the activity of the particular substance added.

The reduction of the consistency of the heavy medium as enabled by the invention does not only increase the precision of separation but also the throughput rate, mainly where fine grained material down to ca. 1 mm. is separated, because even the finest parts of the heavy component of the feed sink down quickly in the highly fluid medium.

Another special advantage of the new process resides in that it facilitates the recovery of the solids from the medium. The heavy solids settle down quickly out of the dilute suspension obtained by sprinkling on the washing screens because its particles tend to floc owing to the addition of the interface-active agents, when the suspension has been diluted to a critical point, which is below the concentration used for the sink float process.

Another application of the new process is found in the making of cement where the starting materials are wet-ground. The addition of the interface-active agents enables a considerable reduction of the water content of the mix obtained by grinding, without impairing its pumpability. Thus the heat consumption in the subsequent thermal treatment of the ground material in the rotary kiln is reduced.

In this connection the simultaneous stabilizing effect of the additives according to the invention is of advantage during the grinding operation, because it causes the coarse particles to sink quickly, so that they remain subjected to the grinding action, whereas the fines remain in suspension.

In the subsequent examples the results achieved with the application of the new process to the sink-float separation are compared with those obtained with the previously usual procedure.

## Example 1

During the conventional sink-float classification of a Ruhr lean coal having a particle size of 1–5 mm. in a barium sulphate suspension having a specific gravity of 1.9 (specific gravity of barium sulphate=3.88, grain size 100% below 0.06 mm.) the yield of float was 60.5%, misyield (related to 100%)=8.74. The yield of sink was 39.5%, misyield (related to 100%)=31.13%.

When 4.5–5.5 kg./m.<sup>3</sup> of coconut amine acetate were added to the heavy medium to reduce its consistency, the quality of the separation was enhanced as follows:

Yield of float 65%, misyield (related to 100%)=0%.  
Yield of sink 35%, misyield (related to 100%)=6.99%.

3  
Example 2

The sink-float classification of the same Ruhr coal of a smaller particle size of 0.5-1 mm, in the same barium sulphate suspension without addition of consistency reducing agent resulted in a yield of float of 58.20%, misyield (related to 100%)=17.55, and a yield of sink of 41.80%, misyield (related to 100%)=57.10%.

After an addition of 4.5-5.5 kg./m.<sup>3</sup> of coconut amine acetate to the barium sulphate suspension the following results were obtained: Yield of float 63.50%, misyield (related to 100%)=0%; yield of sink 36.50%, misyield (related to 100%)=4.27%.

In the foregoing examples the term "misyield" is employed to indicate that portion of the material treated which is not true sink or float material and is considered as a loss unless recycled.

## Example 3

This example illustrates the possibility of making slurries which are suitable for the float and sink separation and have a high specific gravity, containing more than 50% by volume of heavy solids, for the classification of ore.

A slurry made with an eutectic lead-tin alloy having a specific gravity of 8.11 as a heavy solid had ca. 9.0 kg./m.<sup>3</sup> of coconut amine acetate added thereto. This enabled an increase of the heavy-solids content of the slurry to 56% by volume, resulting in a slurry having a specific gravity of 5.02, without impairing the usefulness of the suspension for the separation.

That slurry was used for classifying Kiruna magnetite into low-phosphorus and high-phosphorus components.

Initially that magnetite floated entirely in the suspension having the specific gravity 5.02. After a small reduction of the specific gravity only the high-phosphorus component of the ore floated.

Numerically the result was as follows:

|            | Percent<br>by<br>Weight | Percent<br>Fe | Percent<br>P | Yield of— |       | 40 |
|------------|-------------------------|---------------|--------------|-----------|-------|----|
|            |                         |               |              | Fe        | P     |    |
| Feed.....  | 100.0                   | 42.8          | 0.033        | 100.0     | 100.0 |    |
| Sink.....  | 61.0                    | 59.7          | 0.010        | 85.0      | 18.0  |    |
| Float..... | 39.0                    | 16.4          | 0.070        | 15.0      | 82.0  | 45 |

## Example 4

This example illustrates the advantageous influence of the new process on the clarification or thickening of the thin slurry sprinkled from the screened material and containing the heavy solids.

An untreated barium sulphate suspension used for a float and sink separation was diluted on the washing screens by the sprinkling water so that the passing liquid had a solids content of 70 grams per liter.

The solids did not settle out appreciably from this thin slurry within 30 seconds.

After 8.5-9.0 kg./m.<sup>3</sup> coconut amine acetate was added the thin slurry had clarified almost completely after 30 seconds as a result of the flocculation.

The foregoing examples of applications for the new process in various fields could be amplified as desired in the sense of the general statements hereinbefore.

What is claimed is:

- 10 1. In a sink-float separation process in which an aqueous suspension of a heavy solid is employed as a heavy medium for such separation, the step which comprises incorporating an alkyl amino compound selected from the group consisting of alkyl amines of the formula  $C_nH_{2n+1}NH_2$ , in which  $n$  is an integer between 6 and 18 and their salts in the aqueous suspension of the heavy solid employed for such separation medium to reduce the apparent viscosity thereof, the quantity of heavy solid in said suspension being so high that in the absence of said amino compound its apparent viscosity would be too great for use as a sink-float separation medium.
- 15 2. The process of claim 1 in which the quantity of alkyl amino compound incorporated in the suspension is from 1 to 20 kg. per cubic meter of suspension.
- 20 3. The process of claim 1 in which a mixture of such alkyl amino compounds is incorporated in the suspension.
- 25 4. The process of claim 1 in which said alkyl amino compound is a coconut amino compound.

## References Cited in the file of this patent

## UNITED STATES PATENTS

|           |                 |                |
|-----------|-----------------|----------------|
| 2,108,495 | Levin           | Feb. 15, 1938  |
| 2,286,835 | Robinson et al. | June 16, 1942  |
| 2,309,931 | Cameron         | Feb. 2, 1943   |
| 2,320,009 | Ralston et al.  | May 25, 1943   |
| 2,331,049 | Schindler       | Oct. 5, 1943   |
| 2,468,657 | Dyke et al.     | Apr. 26, 1949  |
| 2,568,992 | Descher         | Sept. 25, 1951 |
| 2,589,949 | Meadors         | Mar. 18, 1952  |
| 2,599,342 | Meadors         | June 3, 1952   |
| 2,719,610 | Erickson        | Sept. 27, 1955 |

## FOREIGN PATENTS

|         |               |               |
|---------|---------------|---------------|
| 830,341 | France        | May 9, 1938   |
| 532,103 | Great Britain | Jan. 17, 1941 |

## OTHER REFERENCES

Armeens: Booklet pub. by Armour Chem. Div., Armour and Co., Chicago, Ill., August 1949, 6 pp.

McCray: Chemistry and Control of Lime Base Muds, article in The Petroleum Engineer, November 1949, pp. B-54, B-56 and B-58.